

G. A. LUTZ.

METHOD OF PROTECTING CONDUITS FOR ELECTRIC CONDUCTORS.

APPLICATION FILED JAN. 19, 1909.

1,072,478.

Patented Sept. 9, 1913.



Witnesses:

John W. Wainwright

Marie F. Wainwright

Inventor  
George A. Lutz.  
By his Attorney, T. F. Bourne

# UNITED STATES PATENT OFFICE.

GEORGE A. LUTZ, OF PLAINFIELD, NEW JERSEY, ASSIGNOR TO AMERICAN CIRCULAR LOOM COMPANY, OF PORTLAND, MAINE, A CORPORATION OF MAINE.

## METHOD OF PROTECTING CONDUITS FOR ELECTRIC CONDUCTORS.

1,072,478.

Specification of Letters Patent.

Patented Sept. 9, 1913.

Application filed January 19, 1909. Serial No. 473,157.

*To all whom it may concern:*

Be it known that I, GEORGE A. LUTZ, a citizen of the United States, and resident of Plainfield, in the county of Union and State 5 of New Jersey, have invented certain new and useful Improvements in Methods of Protecting Conduits for Electric Conductors, of which the following is a specification.

Metal conduits, such as pipes and tubes 10 for electric conductors, outlet boxes, and other fittings used in systems of electrical distribution are liable to become oxidized or rusted in use, and to prevent such rusting and maintain the conductivity of the surface 15 of such pipes and appliances it has been customary to coat the outside or inside surfaces, or both, with a deposit of metal, such as an electrodeposit of zinc. But such coating or deposit does not always cover fully 20 the entire surface of the metal article as spots or places are left unprotected, at which spots the oxidation or rusting can take place. This is due, so far as I am aware, to the fact that the electrodeposit of metal is not sufficiently homogeneous throughout, in that the 25 metal during the process of being deposited becomes more or less rough or pitted, leaving small openings through the deposit.

The object of my invention is to cause the 30 electrodeposit upon the surface of metal, such as galvanizing by the deposit of zinc on the metal, to thoroughly cover the surface of the metal upon which the deposit is placed, to prevent oxidation or rusting 35 thereof.

In carrying out my invention I first thoroughly clean the surface of the metal to be coated, as by pickling, scouring or in any other well known manner, then apply a metallic deposit or coating thereon, preferably 40 by the electroplating process, as by depositing zinc upon such surface, and I then apply pressure to such coating, as by drawing the coated metal article through a die, or by applying such pressure by means of revolving 45 rolls, in contact with such coating or deposit, and if the interior surface of such article is coated with the metal I create pressure thereon by means of a suitable tool, such as a ball or an expanding burnishing tool, either 50 drawn through the article or the article being drawn over the same. In the case of a

pipe, where its interior and exterior surfaces are coated with the metal deposit, the pressure may be applied to the exterior and interior coatings simultaneously by drawing the coated pipe through a die while the burnishing or rubbing tool is, within the pipe, acting on the coating, so that the one passage of the pipe along the die and tool would be 55 sufficient to simultaneously rub or burnish both the exterior and interior coatings of the pipe. The interior and exterior burnishing or rubbing of the metal deposits upon the pipe may be accomplished simultaneously 60 with rotating rolls in contact with the exterior deposit and the ball or similar tool operating upon the deposit upon the interior of the pipe. Such rubbing and burnishing of the metal deposit or coating upon the 65 article causes the metal coating to flow, so that it will be thoroughly smoothed, and will fill spots or places left in the coating while being deposited, thereby causing the coating to be continuous throughout. Such covering 70 of the open spots or places in the electrodeposit upon the metal article protects the same, preventing oxidation or rusting thereat, and producing a more uniform and smooth protecting metallic coating upon and 75 within the metal article.

The accompanying drawing is a partial sectional view, illustrating an electroplated pipe in connection with an external die and interior ball adapted for rubbing and burnishing the metal deposits.

The die A may be of any suitable form, and may be similar to dies used in drawing metal, being shown supported in any suitable support B, the metal coating c upon 90 pipe C being adapted to be drawn and burnished by die A as the pipe is pulled through the die. The coating c<sup>2</sup> upon the inner surface of pipe C is adapted to be drawn and burnished by the tool or ball D within the 95 pipe in contact with the deposit c<sup>2</sup>. The tool D is shown attached to a rod E which may be held in any suitable manner. The arrangement is such that by having the tool D within die A, as shown, the pressure will 100 be uniform, so that when the coated pipe C is pulled through the die both coatings c and c<sup>2</sup> will be operated upon simultaneously.

It is obvious that if the pipe has the ex-

terior coating *c* only the tool *D* may be dispensed with, and if the pipe has the interior coating *c<sup>2</sup>* only the die *A* may be dispensed with. The tool *D* also may be used on the 5 interior of the pipe while rotating rolls in place of the die *A* are used upon the exterior coating *c* of the pipe.

While I have illustrated my improvements in connection with a pipe, it will be understood that outlet boxes, and other fittings 10 for systems of electrical distribution, having an electrodeposit of metal upon the surface or surfaces, may be treated in the manner set forth by any suitable rubbing or burnishing 15 tool.

I have described my invention in connection with pipe and appliances for systems of electrical distribution, but it will be understood that the articles treated are not 20 confined to such use, as articles for other uses may be produced in accordance with my invention.

Having now described my invention what I claim is:

1. The method of protecting articles from 25 oxidation consisting in applying an electrodeposit of metal upon such article, then causing such metal deposit to flow upon the surface of said article to fill spots in such deposit.

2. The method of protecting a metal pipe 30 from oxidation consisting in applying an electrodeposit of metal upon the interior and exterior surfaces of the pipe, and then simultaneously causing said exterior and interior 35 deposits to flow to fill open spots left in said deposits.

Signed at New York city, in the county of New York, and State of New York, this 13th day of January, A. D. 1909.

GEORGE A. LUTZ.

Witnesses:

RALPH H. RAPHAEL,  
T. F. BOURNE.